

# United States Patent Office

3,330,651  
Patented July 11, 1967

1

3,330,651  
FERROUS ALLOYS  
Charles N. Younkin, Unity Township, Westmoreland County, Pa., assignor to Latrobe Steel Company, a corporation of Pennsylvania  
No Drawing. Filed Feb. 1, 1965, Ser. No. 429,660  
4 Claims. (Cl. 75—123)

This invention relates to ferrous alloys and particularly to an improved high manganese wear resistant steel. High manganese steels such as the well-known "Hadfield manganese" type steel have long been known and used for conditions of severe pounding impact and abrasion such as occurs in shot blast and crusher liners, hammers, wearing blades, dredge bucket, switch points, excavating bucket teeth, and the like. It has long been the desire of the industry to provide a steel alloy having improved resistance to the severe pounding impact and abrasion characteristic of the aforementioned uses without the addition of expensive alloying ingredients.

I have discovered an alloy having the resistance to severe pounding impact equivalent to Hadfield manganese type steel together with markedly improved resistance to abrasion. The alloy of my invention otherwise has the standard metallurgical characteristics of Hadfield manganese type steels.

The broad composition of my alloy is:

C—about 1% to about 3%  
Mn—about 10% to about 14%  
Si—2% max.  
Ni—0% to about 4%  
Ti—about 0.5% to about 5%

The balance iron with residual impurities in ordinary amounts, the titanium being combined with carbon in the weight ratio of about 4:1 to form titanium carbide.

While the alloy of this invention may fall within the range of a concentration of alloying elements just enumerated, it is generally desirable to hold the composition within the following somewhat narrower range for maximum effectiveness.

C—about 1.15 to about 2.25%  
Mn—about 12% to about 13%  
Si—about 0.15% to about 0.75%  
Ni—about 0% to about 4%  
Ti—about 0.5% to about 3.5%

The balance iron with residual impurities in ordinary amounts, the titanium being combined with carbon in the weight ratio of about 4:1 as titanium carbide.

The highly advantageous properties of the alloy of this invention will be apparent from the following comparison of a concentration of Hadfield manganese alloy with alloy made according to my invention. The composition of the several alloys are set out in Table I.

TABLE I.—CHEMISTRY

| Alloy Designation | C    | Si  | Mn    | S    | P    | Ti   |
|-------------------|------|-----|-------|------|------|------|
| WR-239            | 1.16 | .22 | 12.65 | .009 | .003 |      |
| WR-240            | 1.26 | .21 | 12.85 | .009 | .002 | .28  |
| WR-241            | 1.37 | .23 | 12.95 | .010 | .002 | .57  |
| WR-242            | 1.41 | .18 | 12.65 | .009 | .002 | .87  |
| WR-282            | 2.19 | .23 | 12.45 | .007 | .003 | 3.80 |
| WR-60068          | 1.46 | .40 | 13.70 | .014 | .003 | 1.27 |

2

Surface hardness and Charpy impact tests were made and the values are set out in the following Table II.

TABLE II.—SURFACE HARDNESS

| 5  | Alloy  | Aust., 1,850° F., $\frac{1}{2}$ Hour Water Quench | After Shot Peening | Charpy Impact As-Quenched |
|----|--------|---------------------------------------------------|--------------------|---------------------------|
| 10 | WR-239 | 187 BHN                                           | 49.0 Rc            | 100+, 240+, 184           |
|    | WR-240 | 212 BHN                                           | 49.0 Rc            | 116, 113, 117             |
|    | WR-241 | 217 BHN                                           | 49.0 Rc            | 95, 91, 88                |
|    | WR-242 | 217 BHN                                           | 49.0 Rc            | 75, 82, 78                |
|    | WR-282 | 279 BHN                                           | 51.0 Rc            |                           |

15 Photomicrographs were made following a standard Nital etch and the structure appears as follows:

TABLE III.—STRUCTURE

| 20 | Alloy  | After 1,850° F., $\frac{1}{2}$ Hour Water Quench  | Approximate Percent TiC (By Area) | ASTM, Grain Size |
|----|--------|---------------------------------------------------|-----------------------------------|------------------|
| 25 | WR-240 | After 1,850° F., $\frac{1}{2}$ Hour Water Quench. | 1                                 | 7                |
|    | WR-241 | do                                                | 1½                                | 7                |
|    | WR-242 | do                                                | 2                                 | 7/8              |

30 Samples of each of the alloys were subject to abrasion tests and the results appear in Table IV.

TABLE IV

| Alloy designation: | Percent improvement in abrasion resistance |
|--------------------|--------------------------------------------|
| WR-240             | 3.6                                        |
| WR-241             | 28.6                                       |
| WR-242             | 31.1                                       |

35 I have found that while the presence of titanium combined with carbon markedly affects the abrasion resistance it does not appear to otherwise affect the other basic metallurgical characteristics of the steel. There is no alteration in hardening characteristics so long as sufficient excess carbon is added to combine with the titanium and leave sufficient carbon for hardening ability. This means that the amount of carbon present in any given alloy should be 40 the amount desired to give a selected hardening ability plus an amount equal to combine with the titanium as titanium carbide in the weight ratio of titanium to carbon of 4:1.

45 While I have described certain present preferred embodiments of my invention, it will be understood that this invention may be otherwise embodied within the scope of the following claims.

I claim:

50 1. An abrasion resisting, high impact resisting alloy consisting essentially of about 1% to about 3% carbon, about 10% to about 14% manganese, about 2% maximum silicon, 0 to about 4% nickel, about 0.5% to 5% titanium and the balance iron with residual impurities in ordinary amounts, said titanium being combined with carbon as titanium carbide.

55 2. An abrasion resisting, high impact resisting alloy consisting essentially of about 1.15% to about 2.25% carbon, about 12% to about 13% manganese, about 0.15% to about 0.75% silicon, 0 to about 4% nickel, about 0.5% to 5% titanium and the balance iron with residual impurities in ordinary amounts, said titanium being combined with carbon as titanium carbide.

60 3. An abrasion resisting, high impact resisting alloy consisting essentially of about 1.5% carbon, about 12% manganese, about 0.25% silicon, about 1.5% titanium and the balance iron with residual impurities in ordinary

70

amounts, said titanium being combined with carbon as titanium carbide.

4. An article made from an alloy consisting essentially of about 1% to about 3% carbon, about 10% to about 14% manganese, about 2% maximum silicon, 0 to about 4% nickel, about 0.5% to 5% titanium and the balance iron with residual impurities in ordinary amounts, said titanium being combined with carbon as titanium carbide and characterized by high resistance to abrasion, high impact resistance and the presence of substantially uniformly distributed titanium carbide.

## References Cited

## UNITED STATES PATENTS

|             |         |            |       |          |
|-------------|---------|------------|-------|----------|
| 846,979     | 3/1907  | Churchwood | ----- | 75—123   |
| 981,575     | 1/1911  | Kohlhaas   | ----- | 75—123   |
| 5 1,111,710 | 9/1914  | Wales      | ----- | 75—123   |
| 2,048,163   | 4/1929  | Pilling    | ----- | 148—31   |
| 2,137,945   | 11/1938 | Mathesius  | ----- | 75—123 X |

HYLAND BIZOT, Primary Examiner.

10 P. WEINSTEIN, Assistant Examiner.